

# UNITED STATES PATENT OFFICE.

FOSTER MILLIKEN, OF LAWRENCE, NEW YORK, ASSIGNOR TO FOSTER MILLIKEN,  
S. FULLERTON WEAVER, AND JAMES M. REPLIER, TRUSTEES.

## ALLOY.

1,377,089.

Specification of Letters Patent.

Patented May 3, 1921.

No Drawing.

Application filed October 8, 1919. Serial No. 329,184.

*To all whom it may concern:*

Be it known that I, FOSTER MILLIKEN, a citizen of the United States, and a resident of Lawrence, in the county of Nassau and State of New York, have invented a new and Improved Alloy, of which the following is a full, clear, and exact description.

The object of the invention is to provide a new and improved alloy characterized by a high resistance to the corrosive influences of acids and capable of withstanding high temperatures.

Another object is to provide an alloy especially serviceable for use in the manufacture of still plugs and other fittings liable to be subjected to the action of acids and high temperatures.

The alloy contains the following metals in substantially the following proportions, namely,

|                                    | Per cent. |
|------------------------------------|-----------|
| Copper                             | 45-55     |
| Nickel                             | 29-35     |
| Lead                               | 1-3       |
| Zinc                               | 5-9       |
| Iron                               | 4-8       |
| Silicon copper (approximately 10%) | 1-3       |

These ingredients are melted together and cast in the usual way, and the alloy resulting therefrom possesses the above mentioned acid resisting quality, and is well adapted for high temperature work. The silicon of the 10% silicon copper remains as one of the constituents of the alloy, and the copper of the silicon copper is taken up by the copper forming the principal ingredient of the alloy.

It is understood that the copper of the silicon copper associates with the other copper and the silicon is present in the alloy from a trace to about 30 per cent.

Having thus described my invention, I claim as new and desire to secure by Letters Patent:

An alloy consisting of the following constituents in approximately the following proportions, namely, copper 45 to 55 per cent., nickel 29 to 35 per cent., lead 1 to 3 per cent., zinc 5 to 9 per cent., iron 4 to 8 per cent. and silicon from a trace to about 30 per cent.

FOSTER MILLIKEN.